

# UNITED STATES PATENT OFFICE.

HENRY K. SANDELL, OF CHICAGO, ILLINOIS, ASSIGNOR TO HERBERT S. MILLS, OF CHICAGO, ILLINOIS.

## METAL COMPOSITION.

1,268,495.

Specification of Letters Patent. Patented June 4, 1918.

No Drawing.

Application filed March 23, 1917. Serial No. 156,973.

*To all whom it may concern:*

Be it known that I, HENRY K. SANDELL, a citizen of the United States, residing at Chicago, in the county of Cook and State 5 of Illinois, have invented a new and useful Improvements in Metal Compositions, of which the following is a specification.

My invention relates to improvements in metal compositions. More particularly the 10 invention is concerned with a metallic alloy comprising nickel and tungsten and containing a considerable percentage of carbon. I find that such a body has peculiar properties which render it specially desirable 15 for use as a contact point for making and breaking electrical circuits.

In order to prepare my new metallic substance the apparatus and procedure fully described in my prior application No. 20 119,656, filed September 12, 1916, may conveniently be employed. In brief, the apparatus in question consists of a carbon block having a trough, or hollow, in its upper surface, which serves as the crucible 25 for the production of the alloy. This crucible is heated by internally developed heat generated by the passage through its walls of an electrical current, which is preferably an alternating current.

30 The metals to be alloyed, *i. e.*, nickel and tungsten, each of which should be in a relatively pure state for the best results, are introduced into the crucible and the latter raised to such a temperature as to cause 35 them to fuse. Powdered amorphous carbon, or powdered graphitic carbon is then introduced into the fused mass, the mass being preferably stirred with a carbon stirring-rod. I also find it of advantage to

40 interrupt the current through the crucible at intervals. Within a very few minutes the molten mass within the crucible solidifies or sets. The process is now at an end and the current may be turned off, the crucible 45 permitted to cool and the block of metal composition removed therefrom. This block may then be machined, ground or otherwise fabricated to produce contact points, or other structural elements.

Although I prefer to stir in finely divided amorphous carbon, or finely divided graphitic carbon, during the heating of the metal within the crucible, this is not essential to the success of the process, since I find that the crucible walls themselves are eaten away 55 during the process, the carbon required for the composition being thus supplied to a large extent by the crucible itself.

I find that by the process above described, I am able to produce a metal composition which is substantially homogenous throughout its mass and which upon analysis shows a percentage of carbon (by weight) of from  $2\frac{1}{2}$  to 7 per cent. For the manufacture of contact points I prefer to use for 60 my metal composition substantially pure nickel and tungsten in about the proportions of 4 parts of nickel to one part of tungsten. The metal composition having these 65 constituents I find to be superior to the composition described in my prior application above referred to, in that it is considerably harder and has a longer life when used as a contact point and subjected to the arcing and sparking which is there met with. 70

75 My new metal composition herein described possesses the peculiarities and advantages of the composition described in my prior application above referred to, and in addition is superior to the last-named composition in the respects pointed out.

80 What I claim as new, and desire to secure by Letters Patent, is:

1. A metal composition comprising substantially an alloy of more than 50 per cent. 85 of nickel and less than 50 per cent. of tungsten carrying upward of 3 per cent. of uncombined carbon.

2. A contact point for making and breaking electrical circuits and comprising substantially an alloy of more than 50 per cent. 90 of nickel and less than 50 per cent. of tungsten carrying upward of 3 per cent. of uncombined carbon.

3. A metal composition comprising substantially an alloy of four parts of nickel and one part of tungsten carrying upward 95 of 3 per cent. of uncombined carbon.

4. A contact point for making and breaking electrical circuits and comprising substantially an alloy of four parts of nickel and one part of tungsten carrying upward of 3 per cent. of uncombined carbon.
5. A cast metal contact point for making and breaking electrical circuits and comprising upward of 70 per cent. of nickel, upward

of 20 per cent. of tungsten, and upward of 3 per cent. of graphitic carbon.

6. A cast metal composition comprising substantially an alloy of upward of 50 per cent. of nickel and less than 50 per cent. of tungsten carrying upward of 3 per cent. of graphitic carbon.

HENRY K. SANDELL.

10